

Oct. 23, 1951

C. H. SPARKLIN

2,572,069

RESISTANCE ELEMENT

Original Filed Jan. 15, 1947

2 SHEETS—SHEET 1



INVENTOR:  
Charles H. Sparklin,  
By Schroeder, Merritt,  
Hoffman & Brady *ATTYS.*

Oct. 23, 1951

C. H. SPARKLIN

2,572,069

RESISTANCE ELEMENT

Original Filed Jan. 15, 1947

2 SHEETS—SHEET 2

FIG. 10.



FIG. 11.



FIG. 13.



FIG. 12.



INVENTOR:  
Charles H. Sparklin,  
By Schroeder, Neuman  
Hofgren and Brady Attys.

## UNITED STATES PATENT OFFICE

2,572,069

## RESISTANCE ELEMENT

Charles H. Sparklin, Chicago, Ill., assignor to  
Birtman Electric Company, a corporation of  
Illinois

Original application January 15, 1947, Serial No.  
722,127, now Patent No. 2,512,692, dated June  
27, 1950. Divided and this application August  
4, 1949, Serial No. 108,614

3 Claims. (Cl. 201—63)

1

This invention relates to a resistance element such as may be used in an electric iron sole plate or the like.

This application is a division of my copending application Serial No. 722,127, filed January 15, 1947, now Patent 2,512,692, issued June 27, 1950, which in turn was a continuation-in-part of my application Serial No. 524,850, filed March 3, 1944, now abandoned.

The resistance element of this invention is of extremely sturdy construction that exhibits extremely long service life when used in electric iron sole plates or the like. Where most resistance elements operate from 50 to 750 hours before failure, while the best elements sometimes have a life as long as 5,000 hours, an electric iron containing in the sole plate the new resistance element described and claimed herein has been operated for 20,000 hours without failure, at which point the test was stopped.

The resistance element will be described in conjunction with an electric iron sole plate containing the same. It is, of course, true that the resistance element will be used in other installations and can be used not only as a heating element but also as a component in an electric circuit to supply resistance to the flow of electricity.

The invention is illustrated in the drawings in which Fig. 1 is a plan view of the sole plate of a preferred form of the iron; Fig. 2 is a section taken along the line 2—2 of Fig. 1; Fig. 3 is a sectional view like Fig. 2 illustrating the first phase of forming the embedded resistance element; Fig. 4 is a similar view illustrating the second step; Fig. 5 is a sectional elevation of a suitable plunger employed in carrying out step 30; Fig. 6 is a view similar to Fig. 4, illustrating the iron after the completion of the third and fourth steps; Fig. 7 is a view of one form of the resistance element; Fig. 8 is a view similar to Fig. 6 and showing the iron after completion of the fifth forming step; Fig. 9 is a sectional elevation illustrating a plunger and stamping employed in the fifth forming step; Fig. 10 is a view illustrating a preferred form of resistance element mounting; Fig. 11 is a detail view of the end of the ceramic device shown in Fig. 10 illustrating the method of introducing the resistance wire into the ceramic core; Fig. 12 is a plan view of the iron with the resistance element installed and attached; and Fig. 13 is a sectional view taken along the line 13—13 in Fig. 10.

The sole plate shown in the drawings and including the new resistance element comprises a metal plate 20 of any suitable metal which may

be, for example, aluminum or steel, upon the upper surface of which is a pair of converging slots 21 and 22 bounded by the integral flanges 23, 24, 25 and 26, which may be formed with 5 the sole plate by a single casting operation. The bottom of each slot is substantially semi-cylindrical, as shown at 27 and 28, the upper edge of the semi-cylinder being approximately level with the normal top of the sole plate.

10 In forming the sole plate, each of the slots is filled to an appropriate point with dry, very finely-powdered, magnesium oxide, zirconium silicate, or other suitable powdered insulating material which has the property of cohering 15 when pressed. The volume of material employed will depend upon the compressibility of the powder and the thickness of refractory and insulating coating desired. Ordinarily the amount used should be such as to form a thin semi-tubular coating having a thickness of from  $\frac{1}{8}$  to  $\frac{1}{4}$  inch. Ordinarily about  $\frac{1}{2}$  inch depth of magnesium oxide powder will produce a coating of suitable thickness upon compression. A layer of this powder 30 is indicated in Fig. 3. The powder is then compressed, for example, by a plunger 31 having a semi-cylindrical head 32 under a pressure of from 2.5 to 6 tons per square inch, for example, 3 tons per square inch. The neck 33 of the plunger extends the complete 20 length of one of the slots 21 or 22 and fits tightly enough therein so that the powder will not be forced out around it. The head 32 is narrower than the neck and forms two longitudinal shoulders 34 and 35 which correspond to the thickness of the coating 36 which is produced upon compression of the powder 30. The operation of the plunger 31 upon the powder in the slots produces a coherent self-sustaining semi-tubular bed of refractory insulating material, as shown in Fig. 35. 40. The resistance element (Fig. 7) comprising the resistance member 40 in the form of a wire arranged in a helix having closely spaced convolutions and preferably formed about a ceramic core or rod 41, is then laid within the bed formed by the coating 36. The resistance member or wire may be of the usual Nichrome wire. The method of embedding which is here employed permits the use of larger wire than is usually employed. A suitable wire has a diameter of 0.028 inch and it may be coiled around a ceramic core having a diameter about  $\frac{1}{4}$  inch in convolutions separated by as little as .020 inch. The ends of the wire, as they extend beyond the ceramic core, are preferably doubled back as indicated at 42. This forms a loop 43 at each end.

45

50

55

of the wire which may be used for attachment to the posts 44 and 45, and also has been found desirable in protecting the wire. The life of the resistance element is considerably greater when the ends of the wire have been doubled back as indicated.

When the resistance element has been inserted upon the bed 36, additional powder 50 is added substantially to fill the slots 21 and 22, as shown in Fig. 6. This powder is suitably the same as the powder employed for the underlying bed. The powder is then compressed under a considerably greater pressure such as 25 to 40 tons per square inch, for example 38 tons per square inch, as shown in Figs. 8 and 9. This last compressing is preferably by the use of a plunger 51 having a neck 52 which presses upon a pressure stamping 53. This stamping is in the form of a boat having the same length as the slots 21 and 22. This boat has a bottom 54, and integral upstanding side walls 55 and 56 which are preferably upturned at an angle slightly less than 90°. The metal of the boat is selected to have considerable resilience so that the side walls 55 and 56 tend to engage the flanges 23 and 24 which form the walls of the slot, and to retain the boat therein. The boat thus acts as a closure member tightly sealing the insulating refractory material within the sole plate. It also acts as a heat distributing member which carries heat radiated or conducted into it from the resistance element into the metal of the sole plate and thus considerably reduces radiation losses to the air.

The bottom layer bed 36 having been compressed under the relatively light pressure of 2.5 to 6 tons per square inch is still deformable under additional pressure. When the resistance element wire 40 and core 41 unit is laid on the bed, covered with powdered insulating material 50, and the powder 50 compressed at a pressure of 25 to 40 tons per square inch, the wire 40 and core 41 is pressed into the bed 36 so that the wire penetrates the bed. The tremendous final pressure makes a unitary rigid insulating structure consisting of the core 41 and the surrounding insulating material with the resistance element 40 rigidly held in the surrounding material. The insulating structure is quite solid and completely fills the spaces between the inner surfaces of the slots 21 and 22 and the stampings 53 so that no air pockets are left to later expand under heat. The resistance element wire is solidly held on all sides so that when heated and cooled it can not move under the forces of expansion and contraction. The insulating material and resistance element wire is, in effect, formed into a unitary solid structure with the sole plate and the resistance element lasts as long as the sole plate itself.

During the formation of the embedded resistance element, the ends of the slots may be closed in any desirable fashion, either by temporary closure members applied individually or collectively to the slots, or by mechanism which may be a permanent part of the pressing apparatus. This closing off of the ends of the slots is facilitated by having the ends parallel and by having the slots of equal length. Thus a single closing off element may be employed at each end if desired.

An electric iron containing the new sole plate has been operated for 20,000 hours without failure, at which point the test was stopped. The ordinary electric iron heating unit operates from 50 to 750 hours before failure, while the best

previous irons with a heating element insulated with solid sheet mica sometimes had a life as long as 5,000 hours. The present structure will last indefinitely even when operated at as much as 2,000 watts. It has been found that where a cast iron sole plate is used with the element, the element may be operated at such a temperature that the cast iron will clinker, and the element will continue to operate.

In Figs. 10 and 11 there is shown a preferred form of resistance element. This comprises a ceramic or other insulating material of considerable strength in the form of an elongated generally cylindrical member 60, at each end of which is a cut-away portion 61 extending from the end of the last helical convolution 62 to the end of the core. The material is cut away on substantially a diameter 63 as shown in Fig. 13, and a feeding hole 64 is formed transversely of the neck 65 remaining. In winding the resistance wire upon the core, the twisted double end 70 of the resistance wire is passed inwardly through the opening 64, as shown in Fig. 11, and is then bent at right angles thereto. This effectively anchors the wire and permits the wire to be wound tightly upon the grooves 62. On the completion of the winding, the residual end of the wire, likewise doubled back upon itself and twisted, is drawn inwardly through the hole 64 and bent axially of the rod.

The foregoing detailed description has been given for clearness of understanding only, and no unnecessary limitations should be understood therefrom.

35 I claim:

1. A resistance element comprising a refractory insulating rod, the rod being cut away at each end on one side of the axis of the rod with a transverse opening being provided at each end 40 through the portion of the rod remaining from the cut away part, and a continuous relatively flexible resistance wire extending outwardly through the transverse opening at one end of the rod and thence bent to pass in helical convolutions around the rod to the opposite end thereof and bent to extend inwardly through the transverse opening at said opposite end, the wire being held tightly in said helical convolutions by its own tensional deformation in said transverse openings, each end of said wire being normally positioned in at least a portion of a cut away part at a corresponding end of the rod.

2. The resistance element of claim 1 wherein each end of the wire is doubled back and twisted upon itself to extend back through the corresponding opening.

3. The resistance element of claim 1 wherein said rod is provided with a helical groove in which said helical convolutions are located, and each end of the wire is doubled back and twisted upon itself to extend back through the corresponding opening.

CHARLES H. SPARKLIN.

#### REFERENCES CITED

The following references are of record in the file of this patent:

#### UNITED STATES PATENTS

| 70              | Number    | Name          | Date           |
|-----------------|-----------|---------------|----------------|
|                 | 1,642,223 | Baker         | Sept. 13, 1927 |
| FOREIGN PATENTS |           |               |                |
| 75              | Number    | Country       | Date           |
|                 | 24,986    | Great Britain | Nov. 14, 1902  |